

Aug. 18, 1953

A. L. SCHOELLERMAN

2,649,128

MEANS AND METHOD OF COLD BENDING SHEET METAL

Filed Feb. 24, 1948

2 Sheets-Sheet 1



INVENTOR.

ALVIN L. SCHOELLERMAN

BY

*Herbert E. Metcalf*  
Attorney

Aug. 18, 1953

A. L. SCHOELLERMAN

2,649,128

MEANS AND METHOD OF COLD BENDING SHEET METAL

Filed Feb. 24, 1948

2 Sheets-Sheet 2

Fig. 4



Fig. 5



Fig. 9



INVENTOR.  
ALVIN L. SCHOELLERMAN

BY

*Albert E. Metcalf*  
Attorney

## UNITED STATES PATENT OFFICE

2,649,128

MEANS AND METHOD OF COLD BENDING  
SHEET METAL

Alvin L. Schoellerman, Los Angeles, Calif., assignor to Northrop Aircraft, Inc., Hawthorne, Calif., a corporation of California

Application February 24, 1948, Serial No. 10,445

2 Claims. (Cl. 153—48)

1

My invention relates to a means and method of bending sheet metal and, more particularly, to a means and method of reducing minimum bend radii when thin sheets of aluminum alloy, such as 75 Stal, are bent in the cold state. The invention is particularly adaptable for use in cold bending aluminum alloy flanges on a power brake, for use in airframe fabrication.

75 Stal aluminum alloy comes in sheet or extruded stock and is, at present, the highest strength aluminum alloy used in the industry. In the designation "75 Stal," "75S" indicates the chemical analysis or alloy which in the present example is: Copper, 1.2—2.0%; iron, .7%; silicon, .5%; manganese, .3%; magnesium, 2.1—2.9%; zinc, 5.1—6.1%; chromium, 0.18—0.4%; titanium, 0.2%; other elements totaling 0.15%; the remainder of the whole being aluminum. The "t" designates that the stock has been fully heat treated; and the "al" (Alclad) indicates that the stock has a surface coating of commercially pure aluminum or an alloy thereof. In strength, 75 Stal tests as follows: Tensile strength, 82,000 p. s. i.; yield strength, 72,000 p. s. i.; shear strength, 46,000—49,000 p. s. i.; Brinell hardness factor of 150 (measured with 10 mm. ball). Further, 75 Stal has an endurance limit of 24,000 p. s. i.

Under normal circumstances, relatively large radii are required to form 75 Stal aluminum alloy sheet, for example, by cold bending. This requires the use of wide flanges to obtain edge distance for rivets, and strength is lost due to large radii. Heretofore, to obtain smaller radii, recourse must be had to the use of annealed stock which is very expensive, or to the use of sheets heated to between 300—400° during forming. This latter method represents an extreme working hazard and the ideal temperatures are difficult to maintain accurately.

Accordingly, it is an object of the present invention to provide a means and method of reducing existing minimum bend radii in unannealed alloy sheet stock when cold forming is practiced.

In the aircraft industry, large numbers of alloy sheet flanges are formed on a power brake utilizing a spaced bottom support for the sheet and then applying pressure from above with a round nose punch, the pressure being applied approximately midway between the lower sheet supports. The punch is machined with the curvature desired in the final bend, which is, in most cases, 90°. In cold forming 75 Stal, for example, there is a minimum bend radius for sheets of various

2

thicknesses where the bend can be safely made. Cold bends on smaller radii cause cracking at the bend and cannot be made with conventional round nose punches.

5 In accordance with the present invention, it was found that actually the bend made in the sheet did not conform to the radius of the round nose punch but was smaller, and it is another object of the present invention to provide a means and method of modifying the nose contour of a cold bending punch to the end that minimum bend radii in sheet stock can be reduced from those heretofore obtained.

The invention can be more fully understood by reference to the drawings in which:

Figures 1—3 inclusive are diagrams showing the action of a round nose punch on sheet stock during the formation of a 90° bend in the sheet.

Figure 4 is a diagram showing a preferred type of punch used to obtain smaller bend radii.

Figure 5 is a diagram showing the permissible variation in the punch contour.

Figures 6—8 inclusive are diagrams showing the action of a punch modified in accordance with the present invention.

Figure 9 is a coordinate diagram showing minimum bend radii for different die radii and different sheet thicknesses.

Figure 10 is a diagram showing the invention as used on an offset punch.

Referring to Figures 1—3 inclusive, showing the action of a conventional round nosed punch on sheet stock when cold formed in a power brake, a lower die 1 is placed on the brake bed having spaced uprights 2 terminating in rounded sheet supporting surfaces 3. Sheet stock 4 is placed on the uprights 2 and a conventional round nosed punch 5 is mounted on the brake to be moved downwardly under power between uprights 2, thus bending the sheet. The lower die 1 and punch 5 are generally longer than the bend length desired to be made in the sheet. The radius in the final bend desired is used for developing the rounded surface of the punch.

In Figure 1 the conventional round nose punch is lowered vertically to start the application of pressure on the sheet 4 at a point A and the sheet bends slightly. In Figure 2 the punch is lowered further to form the sheet at the punch radius and the pressure area widens on both sides of point A. As the full depth of punch penetration is approached, however, I have found that the sheet material leaves the die below point A, the sheet bearing on the punch only on each side of point A as shown in Figure 3. Thus, maximum

## 3

bending stresses are set up at point A and the actual bend made has a smaller radius than the punch. It will be noted in Figure 3 that for a 90° bend, a lesser angle is made to allow for spring-back to 90°. However, this spring-back does not restore the proper radius at A nor does it affect the over-stressing of the sheet at A. These stresses cause cracking and even actual separation of the sheet below the minimum bend radius, as has been determined by experience with sheets of different thicknesses and compositions. In other words, almost the entire bending stress is concentrated at or near point A and this causes failure at that point at definite minimum radii.

I have found, however, that by suitably modifying the punch contour that the bending stresses can be distributed over a wider area, thus permitting bends of smaller radii to be cold formed. In addition, this same modification will cause the sheet to more closely assume the radius machined on the punch.

A punch modified in accordance with the present invention is shown in Figure 4 where the end of the punch 5 has lateral surfaces 6 rounded to a desired radius R and then has a flat 7 of extent X formed on the end thereof normal to the direction of force application. Extensive experimentation has proven that, for minimum radii, there is a correlation between radius R and flat extent X that can be expressed as a preferred relationship for a wide range of sheet thicknesses, as follows

$$X = \frac{106R}{125}$$

While the above is the preferred relationship, I have found that some variation is allowable as shown in Figure 5. The range can be up to  $\pm .015X$ . The space between lines  $X+$  and  $X-$  showing the useful range of X.

The action of the punch as modified in accordance with the present invention is quite different from that of a round nosed punch, and is shown diagrammatically in Figures 6-8 inclusive, comparable as to general punch position with Figures 1-3 inclusive, respectively.

In Figure 6, the punch, as modified by flat 7 has just started to apply pressure to the sheet 4 and the pressure is applied substantially along the flat. As shown in Figure 7, as the punch moves further downwardly, the sheet material leaves the flat very early in the bending operation creating two pressure areas at areas B and C. The material is then forced to bend at these latter points along the lateral radii of the punch nose, as shown in Figure 8. In this manner, substantially a true radius is formed around the bend and the bending stresses are uniformly distributed.

The reduction in minimum bend radii that can be obtained by cold bending with the punch embodying the present invention shows a striking reduction over those obtained by a conventional round nose punch and is shown in Figure 9 for 75 Stal alloy sheet for various thicknesses. It will be seen that by the use of the flat end nose punch of the present invention, the allowable minimum bend radii curve E is significantly smaller than design allowables for round nose punches curve F. The minimum radii for 100% forming with the punch of the present invention is shown in curve G.

The punch of the present invention can also be applied to offset punches as shown in Figure 10. 75

## 4

Here the flat is machined on the portion of the offset punch first making contact with the sheet.

While I have described my invention as being accomplished by machining a flat on the advancing end of the punch I wish it to be distinctly understood that the use of a leading area on the punch having a radius greater than the radius of the remainder of the punch is satisfactory to perform the invention and is deemed the full equivalent of the flat (infinite radius) within the scope of the appended claims. For example, the invention has been successfully practiced when the advancing larger radius is 1 1/8 or more times the radius of the remainder of the punch. Obviously, however, the flat is easier to machine and is therefore the preferred form.

What is claimed is:

1. In a power brake for cold bending a metal sheet of 75 Stal, and other materials having substantially the same bending, tearing, and rupturing characteristics as 75 Stal, into a curve of the maximum order of 90° and having a true radius of the order of 2.5 to 4 times the thickness of the sheet, the combination comprising: a punch having an end area initially engageable with a sheet to be bent and side areas extending laterally from said end area and subsequently engageable with the sheet, said side areas being curved about a common center to a true radius equal to the desired true radius of the bend to be effected and said end area having a radius ranging from 1 1/8 times said true radius to infinity and a chordal width of

35

106

125

times said true radius plus or minus 1.5%; a pair of sheet supports providing parallel fulcrums spaced a greater distance apart than the major width of said punch between said side areas plus twice the thickness of the sheet; and means for forcing said punch against a sheet bridged across said supports to bend the sheet around said side areas by contact of the sheet solely with said fulcrums and said punch.

2. The method of cold bending a metal sheet of 75 Stal, and other materials having substantially the same bending, tearing, and rupturing characteristics as 75 Stal, into a curve of the maximum order of 90° and having a true radius of the order of 2.5 to 4 times the thickness of the sheet, the step comprising: supporting the sheet on parallel fulcrums spaced apart a distance greater than twice the desired true radius of the bend to be effected plus twice the thickness of the sheet and forcing a punch against the sheet between said fulcrums to bend the sheet by contact solely with said fulcrums and said punch, said punch having an end area initially engageable with the sheet and side areas extending laterally from said end area and subsequently engageable with the sheet, said side areas being curved about a common center to said true radius and said end area having a radius ranging from 1 1/8 times said true radius to infinity and a chordal width of

70

106

125

times said true radius plus or minus 1.5%.

ALVIN L. SCHOELLERMAN.

## References Cited in the file of this patent

## UNITED STATES PATENTS

| Number    | Name       | Date          | Number      |
|-----------|------------|---------------|-------------|
| 387,498   | Dingledine | Aug. 7, 1888  | 1,850,679   |
| 399,630   | Phillips   | Mar. 12, 1889 | 2,031,982   |
| 491,192   | Schoen     | Feb. 7, 1893  | 2,077,335   |
| 527,100   | Armstrong  | Oct. 9, 1894  | 5 2,458,202 |
| 652,658   | Bischoff   | June 26, 1900 | 19,529      |
| 1,256,672 | Forslund   | Feb. 19, 1918 | 10 366,319  |
| 1,314,877 | Langford   | Sept. 2, 1919 | 409,548     |
| 1,593,511 | Spencer    | July 20, 1926 |             |

| Name      | Date          |
|-----------|---------------|
| Leis      | Mar. 22, 1932 |
| Salzman   | Feb. 25, 1936 |
| Leis      | Apr. 13, 1937 |
| Robertson | Jan. 4, 1949  |

## FOREIGN PATENTS

| Country       | Date         |
|---------------|--------------|
| Great Britain | of 1900      |
| Germany       | Jan. 2, 1923 |
| Germany       | Feb. 6, 1925 |